

# United States Patent [19]

Occelli et al.

[11] Patent Number: **4,944,865**

[45] Date of Patent: **Jul. 31, 1990**

[54] **PROCESS FOR CRACKING HIGH METALS  
CONTENT FEEDSTOCKS**

[75] Inventors: **Mario L. Occelli, Allison Park;  
James V. Kennedy, Pittsburgh, both  
of Pa.**

[73] Assignee: **Chevron Research Company, San  
Francisco, Calif.**

[21] Appl. No.: **909,819**

[22] Filed: **Sep. 19, 1986**

## Related U.S. Application Data

[63] Continuation of Ser. No. 640,388, Aug. 13, 1984, abandoned, and a continuation-in-part of Ser. No. 375,379, May 6, 1982, Pat. No. 4,465,588.

[51] **Int. Cl.<sup>5</sup>** ..... C10G 11/18

[52] **U.S. Cl.** ..... 208/121; 208/52 CT;  
208/113; 208/120, 208/149; 502/521

[58] **Field of Search** ..... 208/120, 121, 113, 251 R,  
208/253, 149, 52 CT; 502/521

## References Cited

### U.S. PATENT DOCUMENTS

3,699,037 10/1972 Annesser et al. ..... 208/164

|           |        |                          |           |
|-----------|--------|--------------------------|-----------|
| 4,071,436 | 1/1978 | Blanton, Jr. et al. .... | 208/120   |
| 4,146,463 | 3/1979 | Radford et al. ....      | 502/34    |
| 4,280,898 | 7/1981 | Tatterson et al. ....    | 208/52 CT |
| 4,316,794 | 2/1982 | Schoennagel ....         | 208/120   |
| 4,432,890 | 2/1984 | Beck et al. ....         | 208/120   |
| 4,440,868 | 4/1984 | Hettinger et al. ....    | 502/65    |
| 4,465,588 | 8/1984 | Occelli et al. ....      | 208/113   |
| 4,466,884 | 8/1984 | Occelli et al. ....      | 208/113   |
| 4,515,903 | 5/1985 | Otterstedt et al. ....   | 502/521   |
| 4,743,358 | 5/1988 | Kugler et al. ....       | 208/52 CT |

## FOREIGN PATENT DOCUMENTS

|         |         |                         |         |
|---------|---------|-------------------------|---------|
| 0204543 | 12/1986 | European Pat. Off. .... | 502/521 |
| 2116062 | 9/1983  | United Kingdom ....     | 502/84  |

*Primary Examiner*—Anthony McFarlane  
*Attorney, Agent, or Firm*—T. G. DeJonghe; Q. T. Dickinson

## [57] ABSTRACT

A process for cracking high metals content feedstocks which comprises contacting said feedstocks under catalytic cracking conditions with a novel catalytic cracking composition comprising a solid cracking catalyst and a magnesium oxide diluent.

**6 Claims, 1 Drawing Sheet**



## PROCESS FOR CRACKING HIGH METALS CONTENT FEEDSTOCKS

### REFERENCE TO RELATED APPLICATIONS

This is a continuation of application Ser. No. 640,388, filed on Aug. 13, 1984, now abandoned, and a continuation-in-part of application Ser. No. 375,379, filed May 6, 1982, now U.S. Pat. No. 4,465,588.

### BACKGROUND OF THE INVENTION

#### 1. Field of the Invention

This invention relates to a process for cracking high metals content feedstocks which comprises contacting said charge stock under catalytic cracking conditions with a catalyst composition comprising a solid cracking catalyst and a diluent comprising a magnesium oxide.

#### 2. Description of the Prior Art

U.S. Pat. No. 3,944,482 to Mitchell et al. discloses a process directed to the catalytic cracking of hydrocarbon feeds containing metals using a fluid catalyst having improved metals tolerant characteristics. Bartholic in U.S. Pat. No. 4,289,605 discloses a process for the catalytic cracking of hydrocarbon feeds containing metals using a catalyst composition containing a solid cracking catalyst and calcined microspheres (for example, calcined kaolin clay) having a surface area within the range of 10 to 15 m<sup>2</sup>/gram.

The use of selected metal oxides, such as magnesium oxide, to effect SO<sub>x</sub> scavenging and the complete combustion of CO to CO<sub>2</sub> is described in U.S. Pat. No. 4,146,463 to Radford et al. The metal oxides can be incorporated into the catalyst, deposited onto the catalyst, or mixed with the catalyst.

### SUMMARY OF THE INVENTION

We have found that the catalytic cracking of high metals content feedstocks such as, for example, those containing iron, vanadium, nickel and copper, can be substantially improved by contacting said feedstocks under catalytic cracking conditions with a novel catalyst composition comprising a solid cracking catalyst and a diluent comprising a magnesium oxide compound wherein the concentration of magnesium oxide is sustained so as to maintain a conversion of at least 55 percent in the cracking zone. The improvement resides in the ability of the catalyst system to maintain high conversion of the feedstock even when the catalyst carries a substantially high level of metal contaminants on its surface, for example, up to 5000 ppm of nickel or nickel equivalents, or even higher, or up to 10,000 to 20,000 ppm of vanadium. By "ppm of nickel equivalent" we mean ppm nickel + 0.20 times ppm vanadium. Thus feedstocks having very high metals content can be satisfactorily used herein.

The cracking catalyst component of the novel catalyst composition used in the novel process herein can be any cracking catalyst of any desired type having high activity. By "high activity" we mean catalyst of fresh MAT Activity above about 1.0, preferably up to about 4.0, or even higher, where percent conversion is the difference between the volume of the fresh feed and the volume of the product boiling above 430° F. divided by the volume of the fresh feed multiplied by 100, and where:

$$\text{Activity} = \frac{\% \text{ Conversion}}{100 - \% \text{ Conversion}}$$

5 The "MAT Activity" was obtained by the use of a microactivity test (MAT) unit similar to the standard Davison MAT [see Ciapetta et al., Oil & Gas Journal, 65, 88 (1967)].

Thus, catalytic cracking catalysts suitable for use 10 herein as host catalyst include amorphous silica-alumina catalysts; synthetic mica-montmorillonite catalysts as defined, for example in U.S. Pat. No. 3,252,889 to Capell et al.; and cross-linked clays (see, for example, Vaughn et al. in U.S. Pat. Nos. 4,176,090 and 4,248,739; 15 Vaughn et al. (1980), "Preparation of Molecular Sieves Based on Pillared Interlayered Clays"; *Proceedings of the 5th International Conference on Zeolites*, Rees, L.V., Editor, Heyden, London, pages 94-101; and Lahav et al., (1978) "Crosslinked Smectites I Synthesis and Properties of Hydroxy Aluminum Montmorillonite", *Clay & Clay Minerals*, 26, pages 107-114; Shabtai, J. in U.S. Pat. No. 4,238,364; and Shabtai et al. in U.S. Pat. No. 4,216,188).

20 Preferably, the host catalyst used herein is a catalyst containing a crystalline aluminosilicate, preferably exchanged with rare earth metal cations, sometimes referred to as "rare earth-exchanged crystalline aluminum silicate" or one of the stabilized hydrogen zeolites. Most preferably, the host catalyst is a high activity cracking catalyst.

25 Typical zeolites or molecular sieves having cracking activity which can be used herein as a catalytic cracking catalyst are well known in the art. Suitable zeolites are described, for example, in U.S. Pat. No. 3,660,274 to Blazek et al., or in U.S. Pat. No. 3,647,718 to Hayden et al. The descriptions of the crystalline aluminosilicates in the Blazek et al. and Hayden et al. patents are incorporated herein by reference. Synthetically prepared zeolites are initially in the form of alkali metal aluminosilicates. The alkali metal ions are exchanged with rare earth metal ions to impart cracking characteristics to the zeolites. The zeolites are, of course, crystalline, three-dimensional, stable structures containing a large number of uniform openings or cavities interconnected by smaller, relatively uniform holes or channels. The effective pore size of synthetic zeolites is suitably between six and 15 Å in diameter. The overall formula for the preferred zeolites can be represented as follows:



30 where M is a metal cation and n its valence and x varies from 0 to 1 and y is a function of the degree of dehydration and varies from 0 to 9. M is preferably a rare earth metal cation such as lanthanum, cerium, praseodymium, neodymium or mixtures of these.

35 Zeolites which can be employed herein include both natural and synthetic zeolites. These zeolites include gmelinite, chabazite, dachardite, clinoptilolite, faujasite, heulandite, analcite, levynite, erionite, sodalite, cancrinite, nepheline, lazurite, scolecite, natrolite, offretite, mesolite, mordenite, brewsterite, ferrierite, and the like. The faujasites are preferred. Suitable synthetic zeolites which can be treated in accordance with this invention include zeolites X, Y, A, L, ZK-4, B, EF, R, HJ, M, Q, T, W, Z, alpha and beta, ZSM-types and omega. The term "zeolites" as used herein contemplates not only aluminosilicates but substances in which the

aluminum is replaced by gallium, phosphorus or boron and substances in which the silicon is replaced by germanium.

The preferred zeolites for this invention are the synthetic faujasites of the types Y and X or mixtures thereof.

To obtain good cracking activity the zeolites have to be in a proper form. In most cases this involves reducing the alkali metal content of the zeolite to as low a level as possible. Further, a high alkali metal content reduces the thermal structural stability, and the effective lifetime of the catalyst will be impaired as a consequence thereof. Procedures for removing alkali metals and putting the zeolite in the proper form are well known in the art as described in U.S. Pat. No. 3,537,816.

The crystalline aluminosilicate zeolites, such as synthetic faujasite, will under normal conditions crystallize as regularly shaped, discrete particles of approximately one to ten microns in size, and, accordingly, this is the size range normally used in commercial catalysts. The particle size of the zeolites can be, for example, from about 0.5 to about 10 microns but generally from about 1 to about 2 microns or less. Crystalline zeolites exhibit both an interior and an exterior surface area, with the largest portion of the total surface area being internal. Blockage of the internal channels by, for example, coke formation and contamination by metals poisoning will greatly reduce the total surface area.

Especially preferred as the catalytically active component of the catalyst system claimed herein is a crystalline aluminosilicate, such as defined above, dispersed in a refractory metal oxide matrix, for example, as set forth in U.S. Pat. No. 3,944,482 to Mitchell et al., referred to hereinabove.

The matrix material in the host catalyst can be any well-known heat-stable or refractory metal compounds, for example, metal oxides, such as silica, magnesia, boron, zirconia, or mixtures of these materials or suitable large pore clays, cross-linked clays or mixed oxide combinations.

The particular method of forming the catalyst matrix does not form a part of this invention. Any method which produces the desired cracking activity characteristics can suitably be employed. Large pored refractory metal oxide materials suitable for use as a matrix can be obtained as articles of commerce from catalyst manufacturers or they can be prepared in ways well known in the art such as described, for example, in U.S. Pat. No. 2,890,162, the specification of which is incorporated herein by reference.

The amount of the zeolitic material dispersed in the matrix can suitably be from about 10 to about 60 weight percent, preferably from about 10 to about 40 weight percent, but most preferably from about 20 to about 40 weight percent of the final catalyst. The method of forming the final composited catalyst also forms no part of this invention, and any method well known to those skilled in this art is acceptable. For example, finely divided zeolite can be admixed with the finely divided matrix material, and the mixture spray dried to form the final catalyst. Other suitable methods are described in U.S. Pat. Nos. 3,271,418; 3,717,587; 3,657,154; and 3,676,330; whose descriptions are incorporated herein by reference. The zeolite can also be grown on the matrix material if desired, as defined, for example in U.S. Pat. No. 3,647,718 to Hayden et al., referred to above.

The second component of the catalyst system used herein, as a separate and distinct entity, is a diluent comprising a magnesium oxide compound, and preferably in combination with an inorganic binder to impart density and strength, and maintain particle integrity. The magnesium oxide can be obtained as the calcination product of such commercially available minerals as magnesia ( $MgO$ ), magnesite ( $MgCO_3$ ) or brucite ( $Mg(OH)_2$ ), or as the thermal decomposition product of such magnesium containing salts as magnesium nitrate, magnesium carbonate, or magnesium acetate. The inorganic binder can be those conventionally employed by those skilled in the art, including but not limited to clays such as attapulgite, bentonite (montmorillonite), hectorite, kaolin or sepiolite, or precipitated synthetic binders such as alumina, silica, silica-alumina, or such items of commerce as Catapal  $\text{R}$ , Chlorohydrol  $\text{R}$ , or SMM  $\text{R}$ , or combinations thereof. The weight ratio of the catalytically active component to the magnesium oxide diluent (the second component) is in the range of about 50:50 to about 90:10, more preferably in the range of about 63:35 to about 80:20.

The catalyst composition defined above possesses a high tolerance to metals and thus is particularly useful in the cracking of high metals content charge stocks. Suitable charge stocks include crude oil, residuums or other petroleum fractions which are suitable catalytic cracking charge stocks except for the high metals contents. A high metals content charge stock for purposes of this invention is defined as one having a total metals concentration equivalent to or greater than a value of ten as calculated in accordance with the following relationship:

$$10[Ni] + [V] + [Fe] \geq 10$$

where  $[Ni]$ ,  $[V]$  and  $[Fe]$  are the concentrations of nickel, vanadium and iron, respectively, in parts per million by weight. The process is particularly advantageous when the charge stock metals concentration is equal to or greater than 100 in the above equation. It is to be understood therefore that the catalyst compositions described above can be used in the catalytic cracking of any hydrocarbon charge stock containing metals, but is particularly useful for the treatment of high metals content charge stocks since the useful life of the catalyst is increased. The charge stocks can also be derived from coal, shale or tar sands. Thus charge stocks which have a metals content value of at least about 10 in accordance with the above equation cannot be treated as well as desired economically in commercial processes today due to high catalyst make-up rates, but can now be treated utilizing the catalyst compositions described and claimed herein. Typical feedstocks are heavy gas oils or the heavier fractions of crude oil in which the metal contaminants are concentrated. Particularly preferred charge stocks for treatment using the catalyst composition of this invention include deasphalted oils boiling above about 900° F. (482° C.) at atmospheric pressure; heavy gas oils boiling from about 600° F. to about 1100° F. (343° C. to 593° C.) at atmospheric pressure; atmospheric or vacuum tower bottoms boiling above about 650° F.

The preferred method of operating the process of this invention using the novel catalyst composition is by fluid catalytic cracking. A suitable reactor-regenerator for carrying out a process using the catalyst composition is shown in the attached FIG. 1. The cracking

occurs in the presence of the fluidized catalyst composition defined herein in an elongated reactor tube 10 which is referred to as a riser. The riser has a length to diameter ratio of above 20 or above 25. The charge stock to be cracked is passed through preheater 2 to heat it to about 600° F. (315.6° C.) and is then charged into the bottom of riser 10 through the end of line 14. Steam is introduced into oil inlet line 14 through line 18. Steam is also introduced independently to the bottom of riser 10 through line 22 to help carry upwardly into the 10 riser regenerated catalyst which flows to the bottom of the riser through transfer line 26.

The oil charge to be cracked in the riser is, for example, a heavy gas oil having a boiling range of about 650° F. to about 1100° F. (343° to 593° C.). The steam added to the riser can amount to about 10 weight percent based on the oil charge, but the amount of steam can vary widely. The catalyst employed is the catalyst composition defined above in a fluid form and is added to the bottom of the riser. The riser temperature range is suitably about 900° F. to about 1100° F. (482° C. to 593° C.) and is controlled by measuring the temperature of the product from the riser and then adjusting the opening of valve 40 by means of temperature controller 42 which regulates the inflow of hot regenerated catalyst 15 to the bottom of riser 10. The temperature of the regenerated catalyst is above the control temperature in the riser so that the incoming catalyst contributes heat to the cracking reaction. The riser pressure is between about 10 and about 35 psig. Between about 0 and about 5 percent of the oil charge to the riser can be recycled. The residence time of both hydrocarbon and catalyst in the riser is very small and ranges from about 0.5 to about 5 seconds. The velocity through the riser is about 35 to about 55 feet per second and is sufficiently high so that there is little or no slippage between the hydrocarbon and the catalyst flowing through the riser. Therefore no bed of catalyst is permitted to build up within the riser whereby the density within the riser is very low. The density within the riser is a maximum of about 30 4 pounds per cubic foot at the bottom of the riser and decreases to about 2 pounds per cubic foot at the top of the riser. Since no dense bed of catalyst is permitted to build up within the riser, the space velocity through the 35 riser is unusually high and will have a range between about 100 or about 120 and about 600 weight of hydrocarbon per hour per instantaneous weight of catalyst in the reactor. No significant catalyst buildup within the reactor is permitted to occur, and the instantaneous 40 catalyst inventory within the riser is due to a flowing catalyst to oil weight ratio between about 4:1 and about 15:1, the weight ratio corresponding to the feed ratio.

The hydrocarbon and catalyst exiting from the top of each riser is passed into a disengaging vessel 44. The top of the riser is capped at 46 so that discharge occurs through lateral slots 50 for proper dispersion. An instantaneous separation between hydrocarbon and catalyst occurs in the disengaging vessel. The hydrocarbon which separates from the catalyst is primarily gasoline together with some heavier components and some lighter gaseous components. The hydrocarbon effluent passes through cyclone system 54 to separate catalyst fines contained therein and is discharged to a fractionator through line 56. The catalyst separated from hydrocarbon in disengager 44 immediately drops below the outlets of the riser so that there is no catalyst level in the disengager but only in a lower stripper section 58. Steam is introduced into catalyst stripper section 58

through sparger 60 to remove any entrained hydrocarbon in the catalyst.

Catalyst leaving stripper 58 passes through transfer line 62 to a regenerator 64. This catalyst contains carbon deposits which tend to lower its cracking activity and as much carbon as possible must be burned from the surface of the catalyst. This burning is accomplished by introduction to the regenerator through line 66 of approximately the stoichiometrically required amount of air for combustion of the carbon deposits. The catalyst from the stripper enters the bottom section of the regenerator in a radial and downward direction through transfer line 62. Flue gas leaving the dense catalyst bed in regenerator 64 flows through cyclones 72 wherein catalyst fines are separated from flue gas permitting the flue gas to leave the regenerator through line 74 and pass through a turbine 76 before leaving for a waste heat boiler wherein any carbon monoxide contained in the flue gas is burned to carbon dioxide to accomplish heat recovery. Turbine 76 compresses atmospheric air in air compressor 78 and this air is charged to the bottom of the regenerator through line 66.

The temperature throughout the dense catalyst bed in the regenerator is about 1250° F. (676.7° C.). The temperature of the flue gas leaving the top of the catalyst bed in the regenerator can rise due to afterburning of carbon monoxide to carbon dioxide. Approximately a stoichiometric amount of oxygen is charged to the regenerator, and the reason for this is to minimize afterburning of carbon monoxide to carbon dioxide above the catalyst bed to avoid injury to the equipment, since at the temperature of the regenerator flue gas some afterburning does occur. In order to prevent excessively high temperatures in the regenerator flue gas due to afterburning, the temperature of the regenerator flue gas is controlled by measuring the temperature of the flue gas entering the cyclones and then venting some of the pressurized air otherwise destined to be charged to the bottom of the regenerator through vent line 80 in response to this measurement. The regenerator reduces the carbon content of the catalyst from about 1±0.5 weight percent to about 0.2 weight percent or less. If required, steam is available through line 82 for cooling the regenerator. Makeup catalyst is added to the bottom of the regenerator through line 84. Hopper 86 is disposed at the bottom of the regenerator for receiving regenerated catalyst to be passed to the bottom of the reactor riser through transfer line 26.

While in FIG. 1 it has been shown that the novel catalyst composition herein can be introduced into the system as makeup by way of line 84, it is apparent that the catalyst composition, as makeup, or as fresh catalyst, in whole or in part, can be added to the system at any desirable or suitable point, for example, in line 26 or in line 14. Similarly, the components of the novel catalyst system need not be added together but can be added separately at any of the respective points defined above. The amount added will vary, of course, depending upon the charge stock used, the catalytic cracking conditions in force, the conditions of regeneration, the amount of metals present in the catalyst under equilibrium conditions, etc.

The relative amounts of the catalytically active and diluent components introduced into the system as makeup can be adjusted so as to increase the concentration of the diluent in the riser and in the system as the concentration of metal contaminants in the cracking zone increases. Accordingly, with the diluent acting as

a scavenger for the metal contaminants, preventing such contaminants from reaching the cracking centers of the catalytically active component, the concentration of the diluent in the makeup catalyst can be adjusted so as to maintain a desired conversion, preferably a conversion of at least 55 percent. The concentration of the diluent component in the cracking zone can be adjusted so as to maintain a conversion of at least 55 percent when the cracking catalyst composite (cracking component plus diluent) contains nickel, vanadium and iron contaminant concentrations in the range of 4000 to 20,000 ppm (based upon the weight of the catalyst composite). The diluent is particularly effective in the scavenging of vanadium.

The reaction temperature in accordance with the above described process is at least about 900° F. (482° C.). The upper limit can be about 1100° F. (593.3° C.) or more. The preferred temperature range is about 950° F. to about 1050° F. (510° C. to 565.6° C.). The reaction total pressure can vary widely and can be, for example, about 5 to about 50 psig (0.34 to 3.4 atmospheres), or preferably, about 20 to about 30 psig (1.36 to 2.04 atmospheres). The maximum residence time is about 5 seconds, and for most charge stocks the residence time will be about 1.5 to about 2.5 seconds or, less commonly, about 3 to about 4 seconds. For high molecular weight charge stocks, which are rich in aromatics, residence times of about 0.5 to about 1.5 seconds are suitable in order to crack mono- and di aromatics and naphthenes which are the aromatics which crack most easily and which produce the highest gasoline yield, but to terminate the operation before appreciable cracking of polycyclic aromatics occurs because these materials produce high yields of coke and C<sub>2</sub> and lighter gases. The length to diameter ratio of the reactor can vary widely, but the reactor should be elongated to provide a high linear velocity, such as about 25 to about 75 feet per second; and to this end a length to diameter ratio above about 20 to about 25 is suitable. The reactor can have a uniform diameter or can be provided with a continuous taper or a stepwise increase in diameter along the reaction path to maintain a nearly constant velocity along the flow path. The amount of diluent can vary depending upon the ratio of hydrocarbon to diluent desired for control purposes. If steam is the diluent employed, a typical amount to be charged can be about 10 percent by volume, which is about 1 percent by weight, based on hydrocarbon charge. A suitable but non-limiting proportion of diluent gas, such as steam or nitrogen, to fresh hydrocarbon feed can be about 0.5 to about 10 percent by weight.

The catalyst particle size (of each of the two components, that is, of the catalytically-active component and of the diluent) must render it capable of fluidization as a disperse phase in the reactor. Typical and non-limiting fluid catalyst particle size characteristics are as follows:

| Size (Microns) | 0-20 | 20-45 | 45-75 | >75   |
|----------------|------|-------|-------|-------|
| Weight percent | 0-5  | 20-30 | 35-55 | 20-40 |

These particle sizes are usual and are not peculiar to this invention. A suitable weight ratio of catalyst to total oil charge is about 4:1 to about 25:1, preferably about 6:1 to about 10:1. The fresh hydrocarbon feed is generally preheated to a temperature of about 600° F. to about 700° F. (316° C. to 371° C.) but is generally not vaporized during preheat and the additional heat required to

achieve the desired reactor temperature is imparted by hot, regenerated catalyst.

The weight ratio of catalyst to hydrocarbon in the feed is varied to affect variations in reactor temperature. Furthermore, the higher the temperature of the regenerated catalyst the less catalyst is required to achieve a given reaction temperature. Therefore, a high regenerated catalyst temperature will permit the very low reactor density level set forth below and thereby help to avoid back mixing in the reactor. Generally catalyst regeneration can occur at an elevated temperature of about 1250° F. (676.6° C.) or more to reduce the level of carbon on the regenerated catalyst from about 0.6 to about 1.5, generally about 0.05 to 0.3 percent by weight. At usual catalyst to oil ratios in the feed, the quantity of catalyst is more than ample to achieve the desired catalytic effect and therefore if the temperature of the catalyst is high, the ratio can be safely decreased without impairing conversion. Since zeolitic catalysts, for example, are particularly sensitive to the carbon level on the catalyst, regeneration advantageously occurs at elevated temperatures in order to lower the carbon level on the catalyst to the stated range or lower. Moreover, since a prime function of the catalyst is to contribute heat to the reactor, for any given desired reactor temperature the higher the temperature of the catalyst charge, the less catalyst is required. The lower the catalyst charge rate, the lower the density of the material in the reactor. As stated, low reactor densities help to avoid backmixing.

The reactor linear velocity while not being so high that it induces turbulence and excessive backmixing, must be sufficiently high that substantially no catalyst accumulation or buildup occurs in the reactor because such accumulation itself leads to backmixing. (Therefore, the catalyst to oil weight ratio at any position throughout the reactor is about the same as the catalyst to oil weight ratio in the charge.) Stated another way, catalyst and hydrocarbon at any linear position along the reaction path both flow concurrently at about the same linear velocity, thereby avoiding significant slippage of catalyst relative to hydrocarbon. A buildup of catalyst in the reactor leads to a dense bed and backmixing, which in turn increases the residence time in the reactor, for at least a portion of the charge hydrocarbon induces aftercracking. Avoiding a catalyst buildup in the reactor results in a very low catalyst inventory in the reactor, which in turn results in a high space velocity. Therefore, a space velocity of over 100 to 120 weight of hydrocarbon per hour per weight of catalyst inventory is highly desirable. The space velocity should not be below about 35 and can be as high as about 500. Due to the low catalyst inventory and low charge ratio of catalyst to hydrocarbon, the density of the material at the inlet of the reactor in the zone where the feed is charged can be only about 1 to less than 5 pounds per cubic foot, although these ranges are non-limiting. An inlet density in the zone where the low molecular weight feed and catalyst is charged below about 4 pounds per cubic foot is desirable since this density range is too low to encompass dense bed systems which induce backmixing. Although conversion falls off with a decrease in inlet density to very low levels, it has been found the extent of aftercracking to be a more limiting feature than total conversion of fresh feed, even at an inlet density of less than about 4 pounds per cubic foot. At the outlet of the reactor the density will be about

half of the density at the inlet because the cracking operation produces about a four-fold increase in mols of hydrocarbon. The decrease in density through the reactor can be a measure of conversion.

The above conditions and description of operation are for the preferred fluid bed riser cracking operation. For cracking in the older conventional fluid bed operation or in a fixed-bed operation, the particular reaction conditions are well known in the art.

### DESCRIPTION OF PREFERRED EMBODIMENTS

A number of runs were carried out wherein a number of diluent-containing catalysts were evaluated for their metals tolerance and compared with the results obtained using a commercial cracking catalyst. The catalysts used in the tests included a commercial FCC catalyst frequently employed for resid cracking (Catalyst 1) alone and physical mixtures of Catalyst 1 and varying concentrations of the magnesium oxide diluent as hereafter described.

The magnesium oxide was obtained by thermally decomposing a reagent grade magnesium nitrate salt ( $Mg(NO_3)_2 \cdot 6H_2O$ ) at 1000° F. (538° C.) and grinding to a fine grained MgO flour (-100 mesh). The magnesium oxide was then intimately admixed with Catalyst 1, so as to obtain blends of host catalyst with MgO at weight ratios of 90:10 (Catalyst 2), 83.4:16.6 (Catalyst 3), 80:20 (Catalyst 4) and 70:30 (Catalyst 5), respectively.

Each catalyst admixture was heat shocked at 1100° F. (593° C.) for one hour, contaminated with vanadium by impregnation with vanadium naphthenates, followed by calcination at 1000° F. (538° C.) for 10 hours and a steam treatment at 1350° F. (732.3° C.) with about 100 percent steam for 14 hours.

All catalyst samples were tested at 960° F. (516° C.) reaction temperature; 16 weight hourly space velocity; 80 seconds of catalyst contact time; and a catalyst to oil ratio of 3.0 with 2.5 grams of catalyst. The charge stock was a gas oil having a boiling range as characterized in Table I below.

TABLE I

| GAS OIL INSPECTIONS                |       | MAT Feedstock |
|------------------------------------|-------|---------------|
| Stock Identification               |       |               |
| Inspections:                       |       |               |
| Gravity, °API, D-287               | 27.9  |               |
| Pour Point, D97, °F.               | 100   |               |
| Nitrogen, wt %                     | 0.09  |               |
| Sulfur, wt %                       | 0.59  |               |
| Carbon Res., D524, wt %            | 0.33  |               |
| Aniline Point, °F.                 | 190.2 |               |
| Nickel, ppm                        | 0.3   |               |
| Vanadium, ppm                      | 0.3   |               |
| Distillation, D1160 at 760 mm, °F. |       |               |
| 10 Pct. Cond.                      | 595   |               |
| 30 Pct. Cond.                      | 685   |               |
| 50 Pct. Cond.                      | 765   |               |
| 70 Pct. Cond.                      | 846   |               |
| 90 Pct. Cond.                      | 939   |               |
| Approx. Hydrocarbon                |       |               |
| Type Analysis, vol %               |       |               |
| Carbon as Aromatics                | 15.6  |               |
| Carbon as Naphthenes               | 21.7  |               |
| Carbon as Paraffins                | 62.7  |               |

The results obtained in each run for Catalyst 1 at vanadium loading of 2500 ppm (Catalyst 1a), 5000 ppm (Catalyst 1b), 10,000 ppm (Catalyst 1c) and 20,000 ppm (Catalyst 1d) are shown below in Table II:

TABLE II

| Catalyst                         | 1      | 1a     | 1b     | 1c     | 1d     |
|----------------------------------|--------|--------|--------|--------|--------|
| Vanadium, ppm                    | 0      | 2500   | 5000   | 10,000 | 20,000 |
| Conversion, vol %                | 79.50  | 71.77  | 65.12  | 43.76  | 24.42  |
| Product Yields, vol %            |        |        |        |        |        |
| Total C <sub>3</sub> 's          | 9.39   | 7.53   | 5.88   | 3.27   | 1.72   |
| Propane                          | 2.02   | 1.73   | 1.19   | 0.58   | 0.56   |
| Propylene                        | 7.38   | 5.81   | 4.69   | 2.68   | 1.16   |
| Total C <sub>4</sub> 's          | 15.98  | 12.67  | 9.61   | 4.10   | 0.94   |
| I-Butane                         | 7.70   | 5.58   | 3.47   | 0.89   | 0.00   |
| N-Butane                         | 1.72   | 1.28   | 0.82   | 0.31   | 0.13   |
| Total Butenes                    | 6.56   | 5.81   | 5.32   | 2.90   | 0.82   |
| C <sub>5</sub> -430° F. Gasoline | 59.52  | 56.28  | 52.01  | 34.30  | 16.66  |
| 430-650° F. LCGO                 | 15.09  | 20.35  | 23.34  | 29.64  | 30.74  |
| 650° F. + DO                     | 5.41   | 7.89   | 11.54  | 26.60  | 44.84  |
| C <sub>3</sub> + Liq. Rec.       | 105.39 | 104.72 | 102.38 | 97.91  | 94.90  |
| FCC Gaso. + Alk.                 | 84.07  | 76.76  | 69.69  | 44.16  | 20.14  |
| Product Yields, wt %             |        |        |        |        |        |
| C <sub>2</sub> and Lighter       | 2.35   | 2.47   | 2.52   | 2.41   | 2.05   |
| H <sub>2</sub>                   | 0.17   | 0.53   | 0.74   | 0.78   | 0.80   |
| Methane                          | 0.72   | 0.70   | 0.62   | 0.62   | 0.45   |
| Ethane                           | 0.68   | 0.67   | 0.64   | 0.58   | 0.44   |
| Ethylene                         | 0.79   | 0.57   | 0.52   | 0.44   | 0.37   |
| Carbon                           | 3.81   | 5.30   | 5.47   | 5.82   | 6.13   |
| Wt. Balance                      | 98.56  | 97.96  | 97.77  | 98.79  | 99.60  |

25 MAT evaluation results for Catalysts 2, 3, 4, and 5 are tabulated in the following Tables III through VI, respectively, for vanadium loadings of 3000 ppm (catalyst subscript a), 10,000 ppm (catalyst subscript b), and 20,000 ppm (catalyst subscript c).

TABLE III

| Catalyst                         | 2      | 2a     | 2b     | 2c     |
|----------------------------------|--------|--------|--------|--------|
| Vanadium, ppm                    | 0      | 3000   | 10,000 | 20,000 |
| Conversion, vol %                | 78.45  | 74.75  | 68.65  | 25.62  |
| Product Yields, vol %            |        |        |        |        |
| Total C <sub>3</sub> 's          | 8.77   | 8.31   | 6.37   | 1.53   |
| Propane                          | 1.98   | 1.96   | 1.10   | 0.39   |
| Propylene                        | 6.79   | 6.35   | 5.27   | 1.14   |
| Total C <sub>4</sub> 's          | 16.01  | 14.54  | 11.47  | 1.30   |
| I-Butane                         | 8.00   | 7.06   | 4.61   | 0.15   |
| N-Butane                         | 1.93   | 1.70   | 1.07   | 0.14   |
| Total Butenes                    | 6.08   | 5.78   | 5.79   | 1.01   |
| C <sub>5</sub> -430° F. Gasoline | 65.16  | 60.86  | 54.30  | 19.59  |
| 430-650° F. LCGO                 | 15.39  | 17.27  | 20.33  | 31.82  |
| 650° F. + DO                     | 6.15   | 7.98   | 11.01  | 42.56  |
| C <sub>3</sub> + Liq. Rec.       | 111.48 | 108.96 | 103.49 | 96.80  |
| FCC Gaso. + Alk.                 | 87.83  | 82.24  | 78.83  | 23.37  |
| Product Yields, wt %             |        |        |        |        |
| C <sub>2</sub> and Lighter       | 2.01   | 2.09   | 2.16   | 1.71   |
| H <sub>2</sub>                   | 0.06   | 0.13   | 0.43   | 0.64   |
| Methane                          | 0.56   | 0.62   | 0.60   | 0.40   |
| Ethane                           | 0.60   | 0.61   | 0.57   | 0.38   |
| Ethylene                         | 0.80   | 0.73   | 0.57   | 0.30   |
| Carbon                           | 3.84   | 3.88   | 4.28   | 4.86   |
| Wt. Balance                      | 99.50  | 98.58  | 96.60  | 99.12  |

TABLE IV

| Catalyst                         | 3      | 3a     | 3b     | 3c     |
|----------------------------------|--------|--------|--------|--------|
| Vanadium, ppm                    | 0      | 3000   | 10,000 | 20,000 |
| Conversion, vol %                | 78.92  | 73.69  | 70.96  | 37.24  |
| Product Yields, vol %            |        |        |        |        |
| Total C <sub>3</sub> 's          | 8.80   | 7.43   | 6.39   | 1.96   |
| Propane                          | 2.37   | 1.29   | 0.78   | 0.32   |
| Propylene                        | 6.43   | 6.14   | 5.61   | 1.63   |
| Total C <sub>4</sub> 's          | 15.34  | 13.62  | 12.13  | 2.37   |
| I-Butane                         | 7.83   | 6.16   | 4.93   | 0.44   |
| N-Butane                         | 1.94   | 1.40   | 0.99   | 0.17   |
| Total Butenes                    | 5.57   | 6.06   | 6.21   | 1.76   |
| C <sub>5</sub> -430° F. Gasoline | 62.05  | 59.37  | 59.77  | 31.28  |
| 430-650° F. LCGO                 | 15.78  | 17.75  | 20.15  | 29.51  |
| 650° F. + DO                     | 5.30   | 8.55   | 8.89   | 33.25  |
| C <sub>3</sub> + Liq. Rec.       | 107.27 | 106.73 | 107.33 | 98.36  |
| FCC Gaso. + Alk.                 | 83.19  | 80.88  | 80.66  | 37.26  |
| Product Yields, wt %             |        |        |        |        |

TABLE IV-continued

| Catalyst                   | 3     | 3a    | 3b    | 3c    |
|----------------------------|-------|-------|-------|-------|
| C <sub>2</sub> and Lighter | 1.93  | 2.04  | 1.99  | 1.69  |
| H <sub>2</sub>             | 0.09  | 0.16  | 0.23  | 0.64  |
| Methane                    | 0.52  | 0.60  | 0.55  | 0.39  |
| Ethane                     | 0.57  | 0.58  | 0.57  | 0.36  |
| Ethylene                   | 0.74  | 0.70  | 0.64  | 0.29  |
| Carbon                     | 3.92  | 3.55  | 3.43  | 4.59  |
| Wt. Balance                | 96.16 | 96.78 | 98.62 | 98.41 |

TABLE VI-continued

| Catalyst                   | 5      | 5a    | 5b    | 5c    |
|----------------------------|--------|-------|-------|-------|
| C <sub>2</sub> and Lighter | 1.95   | 2.02  | 1.94  | 1.40  |
| H <sub>2</sub>             | 0.09   | 0.24  | 0.28  | 0.30  |
| Methane                    | 0.56   | 0.56  | 0.53  | 0.38  |
| Ethane                     | 0.60   | 0.58  | 0.53  | 0.37  |
| Ethylene                   | 0.70   | 0.64  | 0.60  | 0.36  |
| Carbon                     | 4.06   | 4.34  | 4.11  | 3.07  |
| Wt. Balance                | 100.56 | 95.46 | 97.33 | 98.50 |

TABLE V

| Catalyst                         | 4      | 4a     | 4b     | 4c     |
|----------------------------------|--------|--------|--------|--------|
| Vanadium, ppm                    | 0      | 3000   | 10,000 | 20,000 |
| Conversion, vol %                | 77.87  | 74.47  | 69.72  | 45.04  |
| <u>Product Yields, vol %</u>     |        |        |        |        |
| Total C <sub>3</sub> 's          | 10.16  | 7.68   | 6.05   | 2.72   |
| Propane                          | 3.85   | 1.41   | 0.79   | 0.31   |
| Propylene                        | 6.31   | 6.27   | 5.26   | 2.41   |
| Total C <sub>4</sub> 's          | 16.26  | 14.48  | 11.88  | 3.98   |
| I-Butane                         | 8.78   | 6.80   | 5.07   | 0.86   |
| N-Butane                         | 2.38   | 1.48   | 1.01   | 0.25   |
| Total Butenes                    | 5.10   | 6.20   | 5.80   | 2.87   |
| C <sub>5</sub> -430° F. Gasoline | 62.62  | 62.42  | 59.34  | 39.08  |
| 430-650° F. LCGO                 | 16.26  | 17.66  | 21.01  | 29.80  |
| 650° F. + DO                     | 5.87   | 7.87   | 9.26   | 25.17  |
| C <sub>3</sub> + Liq. Rec.       | 111.16 | 110.12 | 107.55 | 100.75 |
| FCC Gaso. + Alk.                 | 82.70  | 84.41  | 78.88  | 48.41  |
| <u>Product Yields, wt %</u>      |        |        |        |        |
| C <sub>2</sub> and Lighter       | 2.10   | 1.94   | 1.72   | 1.78   |
| H <sub>2</sub>                   | 0.09   | 0.11   | 0.22   | 0.55   |
| Methane                          | 0.58   | 0.54   | 0.48   | 0.43   |
| Ethane                           | 0.62   | 0.55   | 0.48   | 0.43   |
| Ethylene                         | 0.82   | 0.73   | 0.54   | 0.37   |
| Carbon                           | 4.57   | 3.53   | 3.45   | 3.92   |
| Wt. Balance                      | 99.23  | 99.26  | 98.34  | 98.25  |

TABLE VI

| Catalyst                         | 5      | 5a     | 5b     | 5c     |
|----------------------------------|--------|--------|--------|--------|
| Vanadium, ppm                    | 0      | 3000   | 10,000 | 20,000 |
| Conversion, vol %                | 74.48  | 73.75  | 73.06  | 46.63  |
| <u>Product Yields, vol %</u>     |        |        |        |        |
| Total C <sub>3</sub> 's          | 9.15   | 7.82   | 6.69   | 2.52   |
| Propane                          | 3.52   | 2.21   | 1.12   | 0.00   |
| Propylene                        | 5.63   | 5.61   | 5.57   | 2.52   |
| Total C <sub>4</sub> 's          | 14.64  | 13.42  | 12.67  | 4.26   |
| I-Butane                         | 7.74   | 6.60   | 5.71   | 0.88   |
| N-Butane                         | 2.06   | 1.69   | 1.24   | 0.21   |
| Total Butenes                    | 4.84   | 5.14   | 5.73   | 3.17   |
| C <sub>5</sub> -430° F. Gasoline | 63.17  | 59.06  | 59.76  | 41.84  |
| 430-650° F. LCGO                 | 18.41  | 18.59  | 19.15  | 28.76  |
| 650° F. + DO                     | 7.11   | 7.66   | 7.79   | 24.61  |
| C <sub>3</sub> + Liq. Rec.       | 112.47 | 106.55 | 106.07 | 101.98 |
| FCC Gaso. + Alk.                 | 81.60  | 78.01  | 79.70  | 51.90  |
| <u>Product Yields, wt %</u>      |        |        |        |        |

10 The data clearly demonstrate that at high vanadium contamination, all of the catalysts offer improved conversion and selectivity (higher gasoline, decreased coke and decreased hydrogen-make) when compared with the commercial reference catalyst containing no diluent. Moreover, performance at higher vanadium loadings tends to improve as diluent content increases.

15 Obviously many modifications and variations of the invention, as herein above set forth, can be made without departing from the spirit and scope thereof and, therefore, only such limitations should be imposed as are indicated in the appended claims.

We claim:

20 1. In a process which comprises the cracking, in the absence of added hydrogen, of a vanadium-containing hydrogen feed in a cracking zone under cracking conditions employing a cracking catalyst having high activity; the improvement which comprises combining with said catalyst a diluent consisting essentially of magnesium oxide to form a catalyst composite, said diluent forming a separate and distinct entity within said catalyst composite, and the concentration of said diluent within said composite being adjusted so as to be directly proportional to the concentration of vanadium on said catalyst composite in said cracking zone and wherein said concentration of said diluent is in the range of 20-50 weight percent of said catalyst composite.

25 2. The process of claim 1 wherein said diluent is combined with said cracking catalyst prior to contacting said hydrocarbon feed in said cracking zone.

30 3. The process of claim 1 wherein said diluent is introduced into said cracking zone in combination with said feed.

35 4. The process of claim 2 wherein said cracking catalyst is a catalyst at equilibrium conditions in said cracking zone.

40 5. The process of claim 1 wherein said diluent is combined with said cracking catalyst so as to maintain a conversion of at least 55 percent in said cracking zone.

45 6. The process of claim 1 wherein the concentration of nickel, vanadium and iron contaminants on said catalyst composite is in the range of 4000 to 20,000 ppm.

\* \* \* \* \*